

## UNITED STATES PATENT OFFICE

2,506,847

## STABILIZED MOTOR FUEL

Theodore B. Tom, Hammond, Ind., assignor to  
Standard Oil Company, Chicago, Ill., a corpora-  
tion of Indiana

No Drawing. Application March 26, 1947,  
Serial No. 737,432

8 Claims. (Cl. 44—68)

1

The present invention relates to new and useful compositions of matter, and particularly to stabilized organic substances and to the method of stabilizing organic substances against oxidative deterioration in the presence of metals or metal compounds which catalyze such oxidation, for example copper, vanadium, manganese, cobalt, chromium and the like and compounds thereof. More particularly, the invention is directed to stabilized petroleum products and to the method of stabilizing petroleum products.

Organic materials such as petroleum products, for example motor fuels, naphthas, Diesel fuels, fuel oils, electrical insulating oils, turbine oils, lubricating oils, greases, waxes, asphalts, and compounded lubricants, synthetic hydrocarbon oils, vegetable oils, animal oils, marine oils, vegetable and fruit juices, textile fibers, anti-oxidants, rubber and rubber products, soaps, etc. are susceptible to oxidative deterioration, particularly in the presence of metals which are oxidation catalysts, for example copper, vanadium, cobalt, chromium, etc. and compounds thereof.

An example of such oxidative deterioration is the formation of gum and/or color in storage or in use of certain types of motor fuels, particularly those obtained from cracking processes. In order to inhibit such gum/or color formation, it has been common practice to add to such fuels various types of anti-oxidants such as for example aminophenols, substituted aminophenols, naphthols, aromatic hydroxy compounds, hard wood tar distillates and other known anti-oxidants. It has been observed that when motor fuels containing anti-oxidants are stored in metal containers or come in contact with metal surfaces containing copper or copper alloys, the inhibiting effect of the anti-oxidant is decreased to the point where gum forms in such fuels in spite of any anti-oxidant they may contain. This deterioration of anti-oxidants is also encountered in fuels which have been subjected to the copper chloride sweetening process. Such oxidative catalyzing effect is also encountered in viscous hydrocarbon oils even though they may contain anti-oxidants, such as for example phenyl alpha naphthylamine, cyclo hexylamine, alkyl amines, etc. When oils, for example refrigerator oils, turbine oils, electrical insulating oils, internal combustion engine lubricants, etc. are brought in contact with metals such as for example copper, chromium, vanadium, or compounds thereof, they oxidize with the formation of sludge and/or color.

It is an object of the present invention to provide organic substances resistant to oxidative de-

2

terioration. Another object of the invention is to provide a method of inhibiting the oxidative deterioration of organic substances in the presence of metals or metal compounds which are oxidation catalysts. Another object of the invention is to provide organic compositions containing a class of inhibitors which will inhibit or suppress the activity of oxidation catalysts. A further object is to provide improved petroleum compositions. Still another object of the invention is to provide petroleum products which are resistant to oxidative deterioration. A further object of the invention is to provide a method of inhibiting the oxidative deterioration of petroleum products containing or coming in contact with metals or metal compounds which catalyze such oxidative deterioration. Other objects and advantages of the invention will become apparent from the following description thereof.

I have discovered that the oxidative deterioration of organic substances can be effectively inhibited by adding to such organic substances, for example petroleum products, a small but sufficient inhibiting amount, for example from about 0.0001% to about 5% and preferably from about 0.005% to about .5% of an organo-arsenic compound having the following formula:



in which  $\text{R}_1$  is an organic radical of the group consisting of aliphatic, cyclo-aliphatic, aromatic and heterocyclic radicals and mixtures thereof,  $\text{R}_3$  and  $\text{R}_4$  are hydrogen, and  $\text{X}$  is at least one element of the group consisting of oxygen and sulfur. It is to be understood that the term "organic radicals" used herein includes organic radicals containing substituent groups such as for example oxy, hydroxyl, thio, amino, halogen or other groups.

Specific examples of compounds falling within the above named arsenic compounds are the following:

Organic arsonic acids e. g.:

|                        |                                           |
|------------------------|-------------------------------------------|
| benzylarsonic acid     | tolylarsonic acid                         |
| butylarsonic acid      | hydroxyphenylarsonic acid                 |
| phenylarsonic acid     | terpenylarsonic acid                      |
| allylarsonic acid      | ethoxyphenylarsonic acid                  |
| octylarsonic acid      | 3-amyl-4-hydroxy-phenylarsonic acid, etc. |
| phenylthioarsonic acid |                                           |
| allylthioarsonic acid  |                                           |
| butylthioarsonic acid  |                                           |
| cetylarsonic acid      |                                           |

## Organo thion-arsonic acid e. g.:

hexyl thion-arsonic acid

phenyl thion-arsonic acid, etc.

## Organo thion-thiol-arsonic acid e. g.:

lauryl thion-thiol-arsonic acid

xylyl thion-thiol-arsonic acid, etc.

## Organo-trithio-arsonic acid, e. g.:

butyl-trithio-arsonic acid

phenyl trithio-arsonic acid, etc.

## Organo monothiol-arsonic acid e. g.:

phenyl monothiol-arsonic acid

decyl monothiol-arsonic acid

xylyl monothiol-arsonic acid, etc.

## Organo dithiol-arsonic acid e. g.:

lauryl dithiol-arsonic acid

isoamyl dithiol-arsonic acid

While all of the organo arsenic compounds of the above type are effective inhibitors, it is not to be implied that all are equivalents since the specific activity of the various compounds varies to some extent.

Although the present invention finds application in compositions wherein the organic substance, for example petroleum fractions, constitute a major proportion, that is, more than 50% of the composition, it can also be suitably employed for the stabilization of compositions in which the organic substance susceptible to oxidation constitutes a minor proportion.

The effectiveness of the herein described compounds as inhibitors against oxidative deterioration, particularly in the presence of metal catalysts, is illustrated by the data in Table I. These data were obtained by subjecting a motor fuel containing an anti-oxidant in the presence of a metal or metal compound to the A. S. T. M. test for determining the stability of motor fuels by accelerated oxidation. This test has A. S. T. M. designation D525-42T and is fully described on page 965 of the A. S. T. M. Standards 1942—Part III. In obtaining the data of Table I the control was a motor fuel containing 0.01% butyl aminophenol as the anti-oxidant.

Table I

| Sample No. |                                                    | A. S. T. M. Induction Period, Minutes |                             |                              |
|------------|----------------------------------------------------|---------------------------------------|-----------------------------|------------------------------|
|            |                                                    | No Copper                             | Soluble Copper <sup>1</sup> | Metallic Copper <sup>2</sup> |
| 1          | Control                                            | 635-680                               | 85-100                      | 155                          |
| 2          | Control+0.005% Benzyl-arsonic acid                 |                                       | 465                         |                              |
| 3          | Control+0.005% Butyl-arsonic acid                  |                                       | 570                         |                              |
| 4          | Control+0.025% Phenylarsonic acid                  |                                       | 670                         |                              |
| 5          | Control+0.005% Phenyl-arsonic acid                 |                                       | 845                         | 895                          |
| 6          | Control+0.005% Allyl-arsonic acid                  |                                       | 835                         |                              |
| 7          | Control+0.005% p-hydroxyphenyl-arsonic acid        |                                       | 880                         |                              |
| 8          | Control+0.005% p-ethoxyphenylarsonic acid          |                                       | 790                         |                              |
| 9          | Control+0.005% 3-amyl-4-hydroxy-phenylarsonic acid |                                       | 830                         |                              |
| 10         | Control+0.005% Commercial Deactivator              |                                       | 790                         | 265                          |

<sup>1</sup> Soluble copper-copper oleate (4 mgs. Cu. per liter fuel).<sup>2</sup> Metallic copper-18 inches No. 18 copper wire.

The above data demonstrate the metal deactivating affect of some of the arsenic compounds of the present invention. It will be noted

that whereas the commercial deactivator (Sample 10), a conventional Schiff's base type, was effective in the presence of soluble copper, it was relatively ineffective in the presence of metallic copper, while the organo arsenic compounds are effective in the presence of both soluble and metallic copper, as evidenced by Sample No. 5.

That this deactivation or inhibition is not dependent upon the anti-oxidant present in the fuel tested is demonstrated by the data in Table II obtained by carrying out the above described test with a thermally cracked naphtha containing no anti-oxidant.

Table II

| Sample No. |                                   | A. S. T. M. Induction Period—Minutes |                |
|------------|-----------------------------------|--------------------------------------|----------------|
|            |                                   | No Copper                            | Soluble Copper |
| 1          | Control                           | 200                                  | 80             |
| 2          | Control+0.005% Phenylarsonic acid | 255                                  | 270            |

25 The organo arsenic compounds of the type herein described are also effective in certain types of naphtha and hydrocarbon solvents which are required to pass vigorous copper strip tests such as the A. S. T. M. D-235 test described in the 30 A. S. T. M. Standards 1942, Part III, page 85 under (Method c), or the A. S. T. M. Method D-484 described on page 82 (Method b) of the same A. S. T. M. Standards for 1942. Despite careful treating operations, frequently so-called finished 35 naphthas contain sufficient amounts of sulfur and/or polysulfides to give bad copper strip test results. By adding a small amount of the herein described additive, naphthas which contain sufficient sulfur or polysulfides to prevent them from 40 passing copper strip tests readily passed the test. The effectiveness of these organo arsenic compounds in permitting finished naphthas to pass these copper strip tests under conditions in which they would fail to pass the test without the 45 presence of the additive is shown by the data in Table III. The data in the table were obtained by the D-235 A. S. T. M. (Method supra.). The stages of copper strip corrosion as set forth in parentheses in Table III are based on the following 50 ratings: copper strips were rated according to an arbitrary scale in which 0 represents a perfect strip and 12 a black, highly corroded one with variations in between, the intermediate strips varying from slightly discolored to highly discolored.

Table III

| Sample No. |                                            | Copper Strip Rating          |   |
|------------|--------------------------------------------|------------------------------|---|
|            |                                            | 1                            | 2 |
| 1          | Control                                    | Transparent Black (Stage 9). |   |
| 2          | Control+Commercial Additive                | Silver (Stage 6).            |   |
| 3          | Control+0.005% p-hydroxyphenylarsonic acid | Claret Red (Stage 3).        |   |
| 4          | Control+0.025% p-hydroxyphenylarsonic acid | Perfect (Stage 0).           |   |

The above data clearly demonstrate the ability of organo arsenic compound-naphtha compositions to pass stringent copper strip tests. For this purpose about 0.001% to about 0.5% by weight, preferably from about 0.005% to about 0.1% by weight of the organo arsenic compound can be employed for improving the response of naphthas to copper strip corrosion tests.

While I have described my invention in con-

nection with the stabilization of motor fuels and naphthas, it is not limited thereto but is applicable to the stabilization of organic substances such as those hereinbefore mentioned against oxidative deterioration whether or not such oxidation is accelerated by a metal or a metal compound catalyst. When employed in lubricants such as lubricating oils and greases, turbine oils, electrical insulating oils and the like, the herein described compounds can be used in conjunction with anti-oxidants, anti-rust compounds, pour point depressants, detergents, anti-wear agents, anti-foam agents, extreme pressure additives, bearing corrosion inhibitors, etc.

While I have described the preferred embodiments of my invention and the preferred mode of carrying out the same, it will be readily apparent to those skilled in the art that many variations and modifications may be made without departing from the scope of my invention.

I claim:

1. A hydrocarbon motor fuel containing from about 0.005% to about 0.5% of an organo arsonic acid having the general formula



in which R is an organic radical of the group consisting of an aliphatic radical and an aromatic radical.

2. A motor fuel as described in claim 1 in which the arsonic acid is an aliphatic arsonic acid.

3. A motor fuel as described in claim 2 in which the arsonic acid is allylarsionic acid.

15

4. A motor fuel as described in claim 1 in which the arsonic acid is an aromatic arsonic acid.

5. A motor fuel as described in claim 4 in which the arsonic acid is phenylarsionic acid.

6. A motor fuel as described in claim 4 in which the arsonic acid is p-ethoxyphenylarsionic acid.

7. A motor fuel composition comprising a major proportion of a hydrocarbon motor fuel normally susceptible to oxidative deterioration in the presence of an oxidation catalyst, and from about 0.005% to about 0.5% of an organo arsonic acid having the general formula



in which R is an organic radical selected from the group consisting of an aliphatic radical and an aromatic radical.

20 8. A motor fuel composition as described in claim 5 in which the oxidation catalyst is of the group consisting of copper and a copper compound.

THEODORE B. TOM.

25

#### REFERENCES CITED

The following references are of record in the file of this patent:

#### UNITED STATES PATENTS

| Number       | Name       | Date          |
|--------------|------------|---------------|
| 1,988,176    | Merrill    | Jan. 15, 1935 |
| 2,312,207    | Clayton    | Feb. 23, 1943 |
| 2,346,156    | Farrington | Apr. 11, 1944 |
| 35 2,396,258 | Friedheim  | Mar. 12, 1946 |

30

35